

# UNITED STATES PATENT OFFICE.

MARTIN LUTHER BRICKER, OF CLEVELAND, OHIO.

## CHARGE FOR USE IN TREATING IRON AND STEEL.

No. 999,864.

Specification of Letters Patent. Patented Jan. 19, 1909.

Application filed February 1, 1908. Serial No. 413,765.

To all whom it may concern:

Be it known that I, MARTIN LUTHER BRICKER, a citizen of the United States, and a resident of Cleveland, in the county of 5 Cuyahoga and State of Ohio, have invented a new and Improved Charge for Use in Treating Iron and Steel, of which the following is a full, clear, and exact description.

This invention relates to certain improvements in charges for treating iron or steel in a molten or fluid condition in order to improve the quality and character of the metal, and, at the same time, to improve the castings formed therefrom.

15 More particularly the invention involves a novel charge or flux designed to be added to the molten iron or steel, and which will serve to increase its fluidity, drive off sulfur and other impurities, and to render 20 castings made from the iron or steel stronger, of closer grain and without blow-holes often occurring.

The charge includes among its constituents, lead, sand, and certain organic matters, 25 and is formed at any time prior to its being added to the fluid metal. In making a charge sufficient for a sixty-ton mass of iron, I mix two ounces of arsenic, three ounces of asafetida, one and one-half ounces of sac- 30 charin, and one pound of dry granulated sugar, all in a finely powdered condition. About one-half of the mixture is then sifted or shaken into a mold or hollow made of the required size in sand, and about fourteen 35 pounds of lead melted to a bright cherry red is then poured into the mold. The other half of the mixture is then sifted or shaken over the lead in the mold while it is hot, and sand is shaken over the mixture. When 40 the lead is cooled, the charge is ready for use in connection with a crucible or ladle filled with molten iron or steel. In case the charge is used with gray-iron, about four ounces of the total compound is required for 45 each ton of metal. For malleable iron, about six ounces of the charge is required, and for steel about eight ounces.

Upon inserting the charge into the molten iron or steel, it slowly sinks to the bottom 50 and becomes thoroughly intermixed with the metal. It adds materially to the fluidity, so that it may be used to facilitate the making of castings from a ladleful of metal which has cooled to such an extent that it is

slightly hardened or stiffened. The increasing of the fluidity of the metal permits of the making of castings having fewer or no blow-holes, and castings made from the iron or steel treated in this manner are stronger, of closer grain, and freer from impurities, particularly sulfur. The adding of the charge serves to expel the sulfur in the iron before the metal is poured into the mold for making the casting.

All of the chemical actions which take place in the formation of the charge and the addition thereof to a ladle or crucible of molten iron or steel, are not understood by me at the present time. I am only aware of the improved results obtained by following the course of procedure above outlined.

One of the objects in employing sugar is that when it comes in contact with the molten lead, it partially melts and forms an adhesive which binds the other organic constituents and the arsenic to the lead, and also causes the outer layer of sand to firmly adhere thereto. The sand chills the molten lead, so that the organic constituents do not burn or char but very slightly and not to an extent to prevent their operating in the manner desired. The lead being considerably heavier than the molten iron, serves to take the entire mass to the bottom and to agitate the same, which agitation is also facilitated by the escape of gases from the charge. The sand covering adheres to the charge and forms a scale covering which prevents the charge from melting the instant it comes in contact with the molten iron, and permits the lead to carry the organic constituents beneath the surface and even to the bottom.

Having thus described my invention, I claim as new and desire to secure by Letters Patent:

1. A charge for use in the treatment of iron or steel, including lead, an organic material, and sand.
2. A charge for use in the treatment of iron or steel, comprising a lead casting, a protecting covering of sand, and an organic material serving to hold the sand on the lead.
3. A charge for use in the treatment of iron or steel, including a body having a greater specific gravity and a lower melting point than molten iron or steel, an organic material, and an insulating coating.
4. A charge for use in the treatment of

iron or steel, including a body having a greater specific gravity and a lower melting point than molten iron or steel, and a mixture of arsenic, asafetida, saccharin and sugar.

5. A charge for use in the treatment of iron or steel, including a body having a greater specific gravity and a lower melting point than molten iron or steel, a mixture of 15  
10 arsenic, asafetida, saccharin and sugar, and a protecting coating of insulating material.

6. A charge for use in the treatment of

iron or steel, including a body having a greater specific gravity and a lower melting point than molten iron or steel, an outer protecting coating of sand, and an organic material serving to hold the same on said body.

In testimony whereof I have signed my name to this specification in the presence of two subscribing witnesses.

MARTIN LUTHER BRICKER.

Witnesses:

HARRIET R. BRICKER,  
JOHN N. S. MCLEAN.